

## UNITED STATES PATENT OFFICE.

HENRY M. SCHLEICHER, OF ROOSEVELT, AND HARVEY M. BURKEY, OF PLAINFIELD, NEW JERSEY, ASSIGNORS TO AMERICAN METAL COMPANY, LTD., OF NEW YORK, N. Y., A CORPORATION OF NEW YORK.

## PROCESS OF REFINING LEAD.

No Drawing.

Application filed November 3, 1921. Serial No. 512,630.

*To all whom it may concern:*

Be it known that we, HENRY M. SCHLEICHER and HARVEY M. BURKEY, of Roosevelt, Middlesex County, New Jersey, and Plainfield, Union County, New Jersey, respectively, have invented certain new and useful Improvements in Processes of Refining Lead; and we do hereby declare the following to be a full, clear, and exact description 10 of the invention, such as will enable others skilled in the art to which it appertains to make and use the same.

This invention relates to a process of separating arsenic and antimony and tin from 15 lead and lead alloys such as lead bullion and antimonial or hard lead. The process is also capable of utilization in the removal of sulphur, selenium, tellurium and similar elements which are frequently present in crude 20 lead.

The object of the invention is the provision of a method whereby arsenic and antimony and tin present in lead may be separately recovered.

Another object of the invention is the provision of a method wherein the principal reagent employed is repeatedly returned for further use in the process so that the cost of 25 operation is materially reduced, it being necessary only to supply additional quantities of the reagent to compensate for losses during the operation.

Further objects and advantages of the invention will be apparent as it is better understood by reference to the following specification in which the preferred embodiment 30 of the invention is described.

The use of an alkali metal compound in the separation of arsenic and antimony from 35 crude lead has been heretofore suggested, the process involving the dropping of the molten lead through a molten bath of the alkali metal compound and the subsequent separation of the lead from the alkali metal 40 compound. In this process, the separation is not readily accomplished and it is necessary to destroy a portion of the alkali metal compound which is retained and carried over by the molten lead from the bath. The process 45 described does not accomplish the desired separation of the antimony and arsenic in an effective and satisfactory manner.

It has been discovered that the desired

separation may be accomplished by subjecting the molten lead to an oxidizing condition preferably by blowing air through the molten lead in the presence of a material having an affinity for arsenic, antimony, tin and similar metals present in the lead which are oxidized by the air passing therethrough. 55 Alkali metal compounds, and particularly sodium hydroxide in a molten condition, are suitable materials having the affinity referred to and these materials are preferably applied by maintaining a molten layer there- 60 of upon the bath of molten lead. To prevent cooling the lead, the alkali metal compound is preferably melted before it is applied thereto and similarly the air may be pre- 65 heated with advantage before it is intro- 70 duced to the molten lead.

In carrying out the process, the lead is melted in a suitable furnace or pot and the molten alkali metal compound is supplied thereto in sufficient quantity to provide a 75 layer thereof upon the surface. The furnace is provided with tuyères through which compressed air may be introduced beneath the surface of the molten lead. These tuyères 80 preferably extend into and through the molten lead so that the air is thoroughly disseminated in the bath.

In the course of the process, arsenic, antimony, tin and elements such as sulphur, selenium and tellurium are oxidized while the 85 lead remains unaffected. The oxides, probably on account of their lower specific gravity, rise to the surface of the lead bath and immediately combine with the molten alkali metal compound forming compounds of sodium and arsenic and compounds of sodium and antimony, for example. These arsenic and antimony compounds are absorbed by the excess molten alkali metal compound with the result that the molten layer stiffens 90 perceptibly as the process proceeds. In the course of time, the layer becomes so stiff as to be drawn into an irregular mass on the surface of the lead bath. The layer is then skinned off, and in the event that the removal of arsenic and antimony has not been 100 completed, a fresh layer of molten alkali metal compound is applied and the process is repeated.

The stiffened skimmings may contain over 105 35% of antimony and arsenic, but the pref-

erable practice is to remove the layer of alkali metal compound when it contains in the neighborhood of 30% of arsenic and antimony. It has been determined that with 5 this percentage the layer is still sufficiently fluid to allow prills or small shot consisting of lead to settle therethrough. This lead shot is introduced into the molten layer of alkali metal compound by the bubbling of 10 air through the lead bath, and so long as it may settle through the layer, the shot is not likely to be carried away when the bath is skimmed. Substantially no lead is combined with the alkali metal compound and 15 any lead which is carried over in the form of shot is recovered and returned in accordance with the further procedure as hereinafter described.

The skimmings of alkali metal compound 20 carrying the antimony and arsenic are, while still warm or even hot, introduced into water and thus disintegrated to produce a solution of alkali metal compound containing a relatively small amount of alkali antimony 25 compounds and practically all of the alkali arsenic tin compounds, and an insoluble residue consisting substantially of alkali antimony compounds. The residue is dried and treated in any desired manner and in 30 accordance with practice well understood in the art for the recovery of antimony therefrom. The solution is treated to recover arsenic and tin. The solution is then evaporated preferably by the use of waste heat 35 from a suitable source and the alkali metal compound is returned for further use in treating fresh quantities of crude lead.

According to the preferred embodiment 40 of the invention, the process may be carried out as follows:

The lead alloys such as antimonial lead is melted in an iron or steel pot in a suitable furnace and is heated to a temperature of from 600 to 650° C. which temperature is 45 preferably maintained during the further treatment of the lead. Sodium hydroxide or ordinary caustic soda is melted and a layer thereof amounting to 2½% of the weight of the lead to be treated is applied 50 to the surface of the lead bath. Air is then introduced to the lead bath through the tuyères as hereinbefore described, the operation continuing for approximately one hour or until the layer of caustic soda becomes 55 thickened to the desired point. The layer is then skimmed off and a fresh layer of caustic soda is supplied, the blowing being resumed for a similar period. The alternate blowing and skimming 60 is repeated as often as may be necessary to remove the impurities. The skimmings will be found to contain approximately 30% of antimony, and by the operation described it is possible, for example, to remove 12% 65 of antimony from a ton of antimonial lead

by subjecting it to twelve successive treatments with fifty pounds of caustic soda, each treatment requiring approximately one hour. The lead may thus be freed from antimony, the product being soft lead.

The skimmings are thrown into water as hereinbefore described with the resulting production of a strong caustic soda solution and an insoluble residue. The solution is decanted and the residue is dried and treated for the recovery of antimony or antimony compounds. This residue contains substantially 60% of antimony mostly in pentavalent state, about 18% of sodium oxide and small amounts of iron and 70 lead. Before such treatment any lead shot carried over in the caustic soda may be separated from the residue and returned to the lead bath. The solution is subjected to a suitable procedure to throw out 75 the arsenic and tin which may be worked up to produce arsenic and tin or compounds of these elements. The solution is then evaporated preferably by flue gases from the melting furnace, and when concentrated and fused, the caustic soda is ready for re-use.

If the lead alloy contains arsenic and antimony, the greater part of the arsenic and tin is eliminated in the early part of the process, that is to say, in the first skimmings of 85 caustic soda. Substantially all of the arsenic and tin are soluble so that they are almost completely separated from the antimony.

Any silver which may be present in the 100 lead remains therewith, since it is unaffected by the process and does not enter the skimmings. The silver may be separated from the lead after the completion of the process in accordance with the usual practice.

From the foregoing it will be understood that the method herein described provides for the effective separation of other metals from lead and that the details of the 110 operation are of such a simple character that they may be readily applied in an economical manner to accomplish the desired object. Soft lead may be produced from lead containing considerable quantities of arsenic, tin and antimony at a minimum of expense and without resorting to any expedients involving materials which are handled with difficulty or which introduce losses in the process.

Various changes may be made in the details of the process within the scope of the accompanying claims and without departing from the invention or sacrificing any of the advantages thereof.

We claim:

1. A method of removing antimony, arsenic, tin and similar metals from lead, which comprises subjecting the molten lead alloys at a temperature which materially 130

exceeds its melting point to an oxidizing gas in the presence of a molten material having a selective affinity for the metals present in the lead, and separating the molten material 5 with the antimony, arsenic, tin and similar metals from the lead.

2. A method of removing antimony, arsenic, tin and similar metals from lead, which comprises subjecting the molten lead 10 alloys at a temperature exceeding 600° C. to a current of an oxidizing gas in the presence of a molten material having a selective affinity for the metals present in the lead, and separating the molten material with the 15 antimony, arsenic, tin and similar metals from the lead.

3. A method of removing antimony, arsenic, tin and similar metals from lead, which comprises subjecting the molten lead 20 alloys at a temperature between 600° and 650° C. to an oxidizing gas in the presence of a molten alkali metal compound, and separating the alkali metal compound with the 25 antimony, arsenic, tin and similar metals from the lead.

4. A method of removing antimony from lead, which comprises forcing a current of air through the molten lead alloy at a temperature materially exceeding its melting 30 point in the presence of an alkali metal hydroxide, and separating the alkali metal compound containing antimony from the lead.

5. A method of removing antimony from lead, which comprises forcing a current of air through the molten lead alloy in the presence of an alkali metal compound, separating the alkali metal compound from the lead, and leaching the alkali metal compound 40 to recover the insoluble antimony compounds therefrom.

6. A method of removing arsenic from lead, which comprises forcing a current of air through the molten lead alloy in the presence of an alkali metal compound, separating the alkali metal compound from the lead, leaching the alkali metal compound, and precipitating the arsenic from the solution 45 with a suitable reagent.

50 7. A method of removing antimony and arsenic from lead, which comprises forcing a current of air through the molten lead alloy in the presence of an alkali metal compound, separating the alkali metal compound 55 from the lead, leaching the alkali metal compound, withdrawing the insoluble antimony compounds, and precipitating arsenic com-

pounds from the solution with a suitable reagent.

8. A method of removing antimony, arsenic, tin and similar metals from lead, which comprises covering the molten lead alloy at a temperature which materially exceeds its melting point with a molten layer 60 of an alkali metal compound, forcing air 65 through the mass, and separating the alkali metal compound from the lead.

9. A method of removing antimony, arsenic, tin and similar metals from lead, which comprises covering the molten lead 70 alloy with a molten layer of an alkali metal compound, forcing air through the mass, skimming the alkali metal compound from the lead when the molten layer stiffens, and repeating the operation with fresh alkali 75 metal compound until the impurities are substantially exhausted.

10. A method of removing tin from lead, which comprises forcing a current of air 80 through the molten lead alloy in the presence of an alkali metal compound, separating the alkali metal compound from the lead, leaching the alkali metal compound, and precipitating the tin from the solution with a suitable reagent.

11. A method of separating antimony, arsenic, tin and lead, which comprises forcing a current of air through the molten lead alloy in the presence of an alkali metal compound, separating the alkali metal compound from the lead, leaching the alkali metal compound, withdrawing the insoluble antimony compounds, precipitating the tin compounds from the solution by a suitable 90 reagent and withdrawing the tin compounds 95 from the solution.

12. A method of separating antimony, arsenic, tin and lead, which comprises forcing a current of air through the molten lead alloy in the presence of an alkali metal compound, separating the alkali metal compound from the lead, leaching the alkali metal compound, withdrawing the insoluble antimony compounds, precipitating the tin compounds from the solution by a suitable 100 reagent, withdrawing the tin compounds from the solution, precipitating the arsenic from the solution and withdrawing the arsenic compounds from the solution.

In testimony whereof we affix our signatures.

MENRY M. SCHLEICHER.  
HARVEY M. BURKEY.